

# United States Patent [19]

De Nora et al.

[11] 3,926,751

[45] Dec. 16, 1975

[54] METHOD OF ELECTROWINNING METALS

[75] Inventors: Oronzio De Nora; Giuseppe Bianchi; Antonio Nidola; Giovanni Trisoglio, all of Milan, Italy

[73] Assignee: Electronor Corporation, Panama City, Panama

[22] Filed: Jan. 31, 1975

[21] Appl. No.: 546,112

## Related U.S. Application Data

[62] Division of Ser. No. 361,022, May 17, 1973, Pat. No. 3,878,083.

## Foreign Application Priority Data

May 18, 1972 Italy ..... 24526/72

[52] U.S. Cl..... 204/105 R; 204/290 F

[51] Int. Cl.<sup>2</sup> ..... C25C 1/00; C25B 11/08

[58] Field of Search..... 204/105 R, 290 F

## [56] References Cited

### UNITED STATES PATENTS

3,878,083 4/1975 De Nora et al..... 204/290 F

Primary Examiner—R. L. Andrews  
Attorney, Agent, or Firm—Hammond & Littell

## [57] ABSTRACT

Novel electrode for oxygen evolution comprising an electroconductive base provided with an outer coating containing a mixed crystal material of tantalum oxide and iridium oxide and preparation and use thereof.

## 6 Claims, No Drawings

## METHOD OF ELECTROWINNING METALS

This is a division of Ser. No. 361,022, filed May 17, 1973, now U.S. Pat. No. 3,878,083.

## STATE OF THE ART

In various electrochemical process such as, for example, in the production of chlorine and other halogens, the production of chlorates, the electrolysis of other salts which undergo decomposition under electrolysis conditions and other electrolysis processes, it has recently become commercially possible to use dimensionally stable electrodes in place of graphite. These dimensionally stable electrodes usually have a film forming valve metal base such as titanium, tantalum, zirconium, aluminum, niobium and tungsten, which has the capacity to conduct current in the cathodic direction and to resist the passage of current in the anodic direction and are sufficiently resistant to the electrolyte and conditions used within an electrolytic cell, for example, in the production of chlorine and caustic soda, to be used as electrodes in electrolytic processes. In the anodic direction, however, the resistance of the valve metals to the passage of current goes up rapidly, due to the formation of an oxide layer thereon, so that it is no longer possible to conduct current to the electrolyte in any substantial amount without substantial increase in voltage which makes continued use of uncoated valve metal electrodes in an electrolytic process uneconomical.

It is, therefore, customary to apply electrically conductive electrocatalytic coatings to these dimensionally stable valve metal electrode bases. The electrode coatings must have the capacity to continue to conduct current to the electrolyte over long periods of time without becoming passivated and in chlorine production, must have the capacity to catalyze the formation of chlorine molecules from the chloride ions at an anode. They must be electroconductive and electrocatalytic and must adhere firmly to the valve metal base over long periods of time under cell operating conditions.

The commercially available coatings contain a catalytic metal or oxide from the platinum group metals, i.e., platinum, palladium, iridium, ruthenium, rhodium, osmium and a binding or protective agent such as titanium dioxide, tantalum pentoxide and other valve metal oxides in sufficient amount to protect the platinum group metal or oxide from being removed from the electrode in the electrolysis process and to bind the platinum group metal or oxide to the electrode base. The binding and protective metal oxide is usually in excess of the platinum group metal or oxide. Anodes of this nature have been described in British Pat. No. 1,231,280.

In anodes for the recovering of metals from uses by electrowinning, a continual source of difficulty has been the selection of a suitable material for the anode. The requirements are insolubility, resistance to the mechanical and chemical effects of oxygen liberated on its surface, low oxygen overvoltage, and resistance to breakage in handling. Lead anodes containing 6 to 15 per cent antimony have been used in most plants. Such anodes are attacked by chloride if present in the electrolyte. This is the case at the huge plant at Chuquicamata, Chile, where it is necessary to remove cupric chloride dissolved from the ore by passing the solution over cement copper, reducing the cupric to

insoluble cuprous chloride. At this plant there was also developed an anode of a copper-silicon alloy, called the Chilex anode, used in a portion of the tank-room. It has a longer life but raises the power consumption because of greater resistance and greater oxygen overvoltage.

Attempts to use mixed oxide coatings such as  $\text{RuO}_2$ — $\text{TiO}_2$  for oxygen evolution have not been satisfactory in commercial use because passivation takes place after 200 to 1000 hours of operation at a current density of 1.2 KA per  $\text{m}^2$ . The use of a  $\text{Ta}_2\text{O}_5$ — $\text{RuO}_2$  mixed oxide coating improves the electrocatalytic activity and the life of the anode somewhat but not enough for commercial use. The use of a  $\text{TiO}_2$ — $\text{IrO}_2$  coating has lower electrocatalytic activity.

## OBJECTS OF THE INVENTION

It is an object of the invention to provide a novel anode for oxygen evolution having an outer coating containing a mixed crystal material containing tantalum oxide and iridium oxide.

It is an additional object of the invention to provide a novel electrode with an outer coating of tantalum oxide and iridium oxide doped to improve the catalytic activity for oxygen evolution.

It is another object of the invention to provide novel electrodes having a coating of a mixed crystal to  $\text{Ta}_2\text{O}_5$ — $\text{IrO}_2$  on a valve metal alloy base having improved mechanical stability.

It is a further object of the invention to provide a novel process for the electrowinning of metals.

These and other objects and advantages of the invention will become obvious from the following detail description.

## THE INVENTION

The novel electrodes of the invention are comprised of an electroconductive base provided with a coating over at least a portion of its outer surface of a mixed material of tantalum oxide and iridium oxide. The coating may be as little as 5% of the outer surface of the electrode but preferably covers 50 to 100% of the active face of the electrode. The preferred ratio of tantalum to iridium calculated in percent of metal is 1:1 to 0.34:1.

The electrode base may be made of any electroconductive material such as metals and alloys thereof such as iron, nickel, lead, copper, etc but is preferably a valve metal such as tungsten, titanium, tantalum, niobium, aluminum or zirconium or alloys of 2 or more of said metals. The valve metal bases may be provided with an intermediate layer such as an oxide of the valve metal or a coating of another metal such as platinum group metals. The base may be a valve metal and at least either one metal having a low hydrogen overvoltage such as alloy of titanium with iron, cobalt, nickel, palladium, vanadium or molybdenum, or mixtures of two or more of said metals; or one metal suitable to form with titanium a protective oxide film even in acid solution such as an alloy of titanium with niobium, tantalum, zirconium or mixtures of two or more of said metals.

In a preferred embodiment of the invention, the electroconductive base is an alloy of a valve metal with a platinum group metal which as an improved corrosion resistance to acid electrolytes encountered in the use of the electrodes such as 5 to 15% sulfuric acid or 1 to 5% hydrochloric acid. A particularly useful alloy is titanium containing 0.1 to 0.20% by weight of palladium.

This corrosion resistance of the support of the coating prevents chipping off of the coating even if the anode is immersed for a few hours in an acid electrolyte without anodic polarization.

In a modification of the invention, the coating containing tantalum oxide and iridium oxide can be doped with an oxide of a metal with a valence of less than +4 to increase the catalytic activity for oxygen evolution without adversely effecting the mechanical properties of the coatings.

Without wishing to be limited to the following theoretical discussion, it is believed that the conductivity of the  $Ta_2O_5$ — $IrO_2$  system is of the *n* type and that the addition of the doping metal oxide reverses the type of conductivity from "*n* type" to "*p* type" which improves the anodic process by producing electronic holes.

The doping metal oxide may be present in the coating in amounts ranging from 0.5 to 5.0% preferably 1.5 to 3.0% by weight of the said system calculated as metal. Examples of suitable doping metal oxides are alkaline earth metals such as calcium, magnesium, barium and members of Groups VIII, VI B and VII B of the periodic Table such as cobalt, iron and nickel, chromium, molybdenum, manganese, etc.

The increase in the catalytic activity of the doped coatings is shown by the lower anode potential of doped anodes as compared to undoped anodes after 8000 hours of operation of the anodes under identical working conditions. The doping seems to have no adverse effect on the mechanical properties of the coatings as there is no coating loss in either instance even after 8000 hours operation.

The electrodes of the invention are particularly useful for electrolytic processes such as cathodic protection, electroflotation, organic electrosynthesis such as hydrodimerization of acrylonitrile and most particularly the electrowinning of metals. The said electrodes have a high electrocatalytic activity and a very low passivation rate of a few millivolts per month at a current density of 1.2 to 2.0 KA per  $m^2$  and a negligible weight loss if kept under anodic polarization.

The novel method of the invention for the preparation of the electrodes of the invention comprises applying to an electroconductive electrode base a solution of a thermally decomposable compound of tantalum and a thermally decomposable compound of iridium, drying the coated electrode base by evaporation of the solvent and then heating the dried electrode base in the presence of an oxygen containing gas such as to form the desired electrode.

The heating step is preferably effected at temperatures of 350° to 600°C, the optimum temperature being 500° to 550°C. At temperatures below 350°C, the oxidation is not completed or requires too long heating time and at temperatures about 600°C, the electrode base is likely to be subjected to distortions and/or destruction by the high temperatures.

The preliminary drying step is preferably effected by gentle heating in air to evaporate the solvent and codeposit the metal compounds. However, any convenient procedure may be used to remove the solvent such as standing under reduced pressure.

In a preferred embodiment of the process, the coating is applied in multiple coats with short periods of intermediate heating such as 500° to 550°C for 5 to 15 minutes with a longer final heating after the last coat such as 500° to 550°C for 45 minutes to 1 1/2 hours. The

coating obtained thereby is very adherent and quite uniform.

The electrodes of this invention are particularly useful for electrowinning process used in the production of various metals because they do not add impurities to the bath which deposit on the cathode, with the metals being won, and thereby contaminate the refined metal, as do anodes of for example lead containing antimony and bismuth which give impure cathode refined metals. Moreover, their resistance to the acid solutions and oxygen evolution and their excellent anode potential makes them desirable for this use.

In the following examples there are described several preferred embodiments to illustrate the invention. However, it should be understood that the invention is not intended to be limited to the specific embodiments.

#### EXAMPLE I

24 Titanium plates 10 mm by 10 mm were etched in boiling 20% hydrochloric acid for sixty minutes and were then thoroughly washed with water. The plates were then coated with an aqueous solution of the compositions of Table I in 12 to 15 coats. After the application of each coat, the plates were dried and then heated for 10 minutes at 450°C to 600°C in an oven with forced air circulation and then allowed to air cool. After the last coat, the plates were heated in the oven at the same temperature for 1 hour and were then air cooled. The values of Table I are calculated as weight of free metal. The tantalum chloride was used as a solution in 20% hydrochloric acid.

TABLE I

| Sample No.     | Coating composition<br>in mg. |   | heating temp<br>in °C |
|----------------|-------------------------------|---|-----------------------|
| A <sub>1</sub> | TaCl <sub>5</sub>             | — | 450                   |
| A <sub>2</sub> | IrCl <sub>3</sub>             | — | 500                   |
| A <sub>3</sub> | —                             | — | 550                   |
| A <sub>4</sub> | —                             | — | 600                   |
| B <sub>1</sub> | TaCl <sub>5</sub>             | — | 450                   |
| B <sub>2</sub> | IrCl <sub>3</sub>             | — | 500                   |
| B <sub>3</sub> | —                             | — | 550                   |
| B <sub>4</sub> | —                             | — | 600                   |
| C <sub>1</sub> | TaCl <sub>5</sub>             | — | 450                   |
| C <sub>2</sub> | IrCl <sub>3</sub>             | — | 500                   |
| C <sub>3</sub> | —                             | — | 550                   |
| C <sub>4</sub> | —                             | — | 600                   |
| D <sub>1</sub> | TaCl <sub>5</sub>             | — | 450                   |
| D <sub>2</sub> | IrCl <sub>3</sub>             | — | 500                   |
| D <sub>3</sub> | —                             | — | 550                   |
| D <sub>4</sub> | —                             | — | 600                   |
| E <sub>1</sub> | TaCl <sub>5</sub>             | — | 450                   |
| E <sub>2</sub> | IrCl <sub>3</sub>             | — | 500                   |
| E <sub>3</sub> | —                             | — | 550                   |
| E <sub>4</sub> | —                             | — | 600                   |
| F <sub>1</sub> | TaCl <sub>5</sub>             | — | 450                   |
| F <sub>2</sub> | IrCl <sub>3</sub>             | — | 500                   |
| F <sub>3</sub> | —                             | — | 550                   |
| F <sub>4</sub> | —                             | — | 600                   |

55 The anode potential for each anode was the determined by electrolysis of 10% by weight sulfuric acid at 60°C and a current density of 1.2 KA/m<sup>2</sup>. The initial anode potential (against NHE) and the anode potential after 3000 and 6000 hours was determined and the coating loss was then determined. The values are reported in Table II.

TABLE II

| Sample No.     | Anode Potential V (NHE)<br>initial value | Anode Potential V (NHE)<br>after 3000 hs. | Anode Potential V (NHE)<br>after 6000 hs. | Coating weight loss<br>mg./cm <sup>2</sup> |
|----------------|------------------------------------------|-------------------------------------------|-------------------------------------------|--------------------------------------------|
| A <sub>1</sub> | 1.50                                     | 1.68                                      | 1.77                                      | 0.2                                        |
| A <sub>2</sub> | 1.52                                     | 1.62                                      | 1.70                                      | 0.0                                        |
| A <sub>3</sub> | 1.52                                     | 1.62                                      | 1.70                                      | 0.0                                        |

TABLE II-continued

| Sample No.     | Anode Potential initial value | V (NHE) after 3000 hs. | V (NHE) after 6000 hs. | Coating weight loss mg./cm <sup>2</sup> |
|----------------|-------------------------------|------------------------|------------------------|-----------------------------------------|
| A <sub>1</sub> | 1.52                          | 1.62                   | 1.77                   | 0.0                                     |
| B <sub>1</sub> | 1.51                          | 1.63                   | 1.73                   | 0.6                                     |
| B <sub>2</sub> | 1.51                          | 1.62                   | 1.68                   | 0.0                                     |
| B <sub>3</sub> | 1.52                          | 1.62                   | 1.68                   | 0.0                                     |
| B <sub>4</sub> | 1.51                          | 1.63                   | 1.79                   | 0.0                                     |
| C <sub>1</sub> | 1.50                          | 1.65                   | 1.70                   | 0.3                                     |
| C <sub>2</sub> | 1.51                          | 1.63                   | 1.64                   | 0.0                                     |
| C <sub>3</sub> | 1.52                          | 1.58                   | 1.63                   | 0.0                                     |
| C <sub>4</sub> | 1.52                          | 1.63                   | 1.73                   | 0.0                                     |
| D <sub>1</sub> | 1.49                          | 1.61                   | 1.68                   | 0.5                                     |
| D <sub>2</sub> | 1.50                          | 1.60                   | 1.62                   | 0.0                                     |
| D <sub>3</sub> | 1.52                          | 1.58                   | 1.62                   | 0.0                                     |
| D <sub>4</sub> | 1.52                          | 1.60                   | 1.67                   | 0.0                                     |
| E <sub>1</sub> | 1.52                          | 1.62                   | 1.66                   | 0.2                                     |
| E <sub>2</sub> | 1.50                          | 1.60                   | 1.61                   | 0.0                                     |
| E <sub>3</sub> | 1.52                          | 1.56                   | 1.61                   | 0.0                                     |
| E <sub>4</sub> | 1.52                          | 1.63                   | 1.67                   | 0.5                                     |
| F <sub>1</sub> | 1.48                          | 1.56                   | 1.73                   | 0.9                                     |
| F <sub>2</sub> | 1.47                          | 1.53                   | 1.74                   | 0.6                                     |
| F <sub>3</sub> | 1.47                          | 1.52                   | 1.77                   | 1.2                                     |
| F <sub>4</sub> | 1.49                          | 1.60                   | 1.80                   | 1.3                                     |

The results of Table II show that the electrodes of the invention have high electrocatalytic activity and a very low passivation rate and that the weight loss of the coating is negligible when within the limits of the invention. It should be noted that the ratio of Ta to Ir for samples F<sub>1</sub> to F<sub>4</sub> is about 0.34. Optimum values are obtained in the heating range of 500°-550°C.

## EXAMPLE II

For comparative purposes, electrodes were prepared as follows. Titanium plates 10 mm by 10 mm were etched in boiling 20% hydrochloric acid for sixty minutes and were then thoroughly washed with water. The plates were then coated with an aqueous solution of the compositions of Table III in 12 to 15 coats. After the application of each coat, the plates were dried and then heated for 10 minutes at 450°C to 550°C in an oven with forced air circulation and then allowed to air cool. After the last-coat, the plates were heated in the oven at the same temperature for 1 hour and were then air cooled. The values of Table III are calculated as weight of free metal.

TABLE III

| Sample No. | Coating composition in mg                   | heating temp in °C |
|------------|---------------------------------------------|--------------------|
| 1          | TiCl <sub>3</sub> — 19.5                    | 450                |
| 2          | RuCl <sub>3</sub> ·3H <sub>2</sub> O — 16.0 | 450                |
| 3          | TiCl <sub>3</sub> — 10.7                    | 450                |
| 4          | RuCl <sub>3</sub> ·3H <sub>2</sub> O — 16.0 | 450                |
| 5          | TiCl <sub>3</sub> — 19.5                    | 500                |
| 6          | TiCl <sub>3</sub> — 16.0                    | 550                |
| 7          | TiCl <sub>3</sub> — 19.5                    | 500                |
| 8          | TiCl <sub>3</sub> — 10.7                    | 550                |
|            | IrCl <sub>3</sub> — 16.0                    |                    |

The anode potential for each anode was then determined by electrolysis of 10% by weight sulfuric acid at 60°C at a current density of 1.2 KA/m<sup>2</sup>. The initial anode potential and the anode potential after 600, 1000 or 1200 hours are reported in Table IV. The final loss of the coating was determined at the end of the test.

TABLE IV

| Sample No. | Anode potential (NHE) in Volts after 600 h | 1000 h | 1200 h | coating loss in mg/cm <sup>2</sup> |
|------------|--------------------------------------------|--------|--------|------------------------------------|
| 1          | 1.48                                       | —      | 2.00   | >2.5                               |
| 2          | 1.47                                       | —      | 1.95   | >2.2                               |
| 3          | 1.46                                       | —      | 1.85   | 2.09                               |
| 4          | 1.45                                       | —      | 1.79   | 2.00                               |
| 5          | 1.52                                       | 1.82   | 1.86   | —                                  |
| 6          | 1.52                                       | 1.89   | 1.93   | —                                  |
| 7          | 1.51                                       | 1.81   | 1.85   | —                                  |
| 8          | 1.52                                       | 1.85   | 1.90   | —                                  |

The results of Table IV show that RuO<sub>2</sub>-TiO<sub>2</sub> coated electrodes become passivated after only 1000 hours and the Ta<sub>2</sub>O<sub>5</sub>-RuO<sub>2</sub> coated electrodes are only slightly improved and the TiO<sub>2</sub>-IrO<sub>2</sub> coated electrodes are no better.

## EXAMPLE III

10 plates of titanium plates containing 0.15% of palladium (10 × 10 mm) were sandblasted and then etched in refluxing 20% hydrochloric acid for 60 minutes. The plates were then coated with the compositions of Table V. The compositions were applied in 15 to 20 coats with intermediate heating at 450°C for 10 minutes in an oven with forced air circulation and cooling in air. The final heating was effected at the temperatures in Table V for 1 hour followed by air cooling.

TABLE V

| Sample No. | Coating compositions in mg of free metal |   | Final heating in °C |
|------------|------------------------------------------|---|---------------------|
| AA         | TiCl <sub>3</sub>                        | — | 16+                 |
| BB         | IrCl <sub>3</sub>                        | — | 16                  |
| CC         | TaCl <sub>3</sub>                        | — | 13.10+              |
| DD         | IrCl <sub>3</sub>                        | — | 16.0                |
| EE         | TaCl <sub>3</sub>                        | — | 10.70+              |
| FF         | IrCl <sub>3</sub>                        | — | 16.0                |
| GG         | TaCl <sub>3</sub>                        | — | 8.60+               |
| HH         | IrCl <sub>3</sub>                        | — | 16                  |
| II         | TaCl <sub>3</sub>                        | — | 6.85+               |
| JJ         | IrCl <sub>3</sub>                        | — | 16                  |

The anode potentials and coating weight loss were determined as in Example I and the results are reported in Table VI.

45

TABLE VI

| Sample No. | Anode Potential in V(NHE) |                | Coating weight loss in mg/cm <sup>2</sup> after 2000 hs. |
|------------|---------------------------|----------------|----------------------------------------------------------|
|            | initial value             | after 3000 hs. | after 6000 hs.                                           |
| AA         | 1.52                      | 1.62           | 1.69                                                     |
| BB         | 1.51                      | 1.63           | 1.70                                                     |
| CC         | 1.51                      | 1.62           | 1.68                                                     |
| DD         | 1.52                      | 1.62           | 1.68                                                     |
| EE         | 1.51                      | 1.63           | 1.65                                                     |
| FF         | 1.52                      | 1.58           | 1.64                                                     |
| GG         | 1.50                      | 1.59           | 1.63                                                     |
| HH         | 1.52                      | 1.58           | 1.62                                                     |
| II         | 1.50                      | 1.57           | 1.60                                                     |
| JJ         | 1.52                      | 1.58           | 1.60                                                     |

The results of Table VI show that the electrodes of the invention with a titanium — palladium alloy base have excellent electrocatalytic activity and low passivation rates.

## EXAMPLE IV

65 To demonstrate the improved corrosion resistance of a titanium — palladium alloy, 10 plates made of titanium containing 0.15% by weight of palladium (10 × 10 mm) were sand-blasted and then etched in refluxing

20% hydrochloric acid for 60 minutes. The plates were then coated with the compositions of Table V using the procedure of Example III. The anode potential was determined for each electrode by electrolysis of 10% sulfuric acid at 60°C and a current density of 1.2 KA/m<sup>2</sup>. The initial anode potential and the value after 1000 and 2000 hours and the coating weight loss after 2000 hours was determined. Moreover, the current was halted for 15 minutes in each 24 hour period without removing the electrode from the acid bath. The results are reported in Table VII.

TABLE VII

| Sample No. | Anode Potential V (NHE) |          |          | Coating weight loss in mg/cm <sup>2</sup> |
|------------|-------------------------|----------|----------|-------------------------------------------|
|            | initial value           | 1000 hs. | 2000 hs. |                                           |
| AA         | 1.52                    | 1.66     | 1.68     | 0.2                                       |
| BB         | 1.51                    | 1.66     | 1.67     | 0.3                                       |
| CC         | 1.51                    | 1.57     | 1.62     | 0.3                                       |
| DD         | 1.52                    | 1.58     | 1.60     | 0.3                                       |
| EE         | 1.50                    | 1.56     | 1.58     | 0.3                                       |
| FF         | 1.52                    | 1.56     | 1.58     | 0.3                                       |
| GG         | 1.50                    | 1.55     | 1.56     | 0.3                                       |
| HH         | 1.52                    | 1.54     | 1.56     | 0.3                                       |
| II         | 1.52                    | 1.54     | 1.55     | 0.3                                       |
| JJ         | 1.51                    | 1.55     | 1.55     | 0.3                                       |

The results of Table VII show that the electrodes of the invention having a titanium — palladium alloy base have excellent electrocatalytic activity and low passivation rates and the coating does not chip off even without anodic polarization.

## EXAMPLE V

10 titanium plates (20 × 20 mm) were etched in refluxing 20% hydrochloric acid for 60 minutes and after being thoroughly washed with water, the plates were coated with an aqueous solution containing 2.01 mg (as free metal) of TaCl<sub>5</sub>, 3.2 mg (as free metal) of IrCl<sub>3</sub> and 0.0394 ml of hydrochloric acid. The solution was applied in 12 coats with intermediate heating and cooling and a final heating as described in Example I.

The coated titanium plates were used as anodes in cells for the recovery of zinc from an aqueous electrolyte containing 100 g/liter of Zn SO<sub>4</sub> (as free metal), 10% sulfuric acid and 10 to 50 ppm of glue. The cathode was a pure aluminum sheet with a smooth surface and the electrolyte gap was 10 mm. The current density was 500 A/m<sup>2</sup> and the electrolyte temperature was 35°C. The anode potential, loss of coating, zinc thickness on the cathode and the morphology of the zinc deposit are reported in Table VIII.

TABLE VIII

| Test No. | Anode potential V (NHE) | Coating weight loss | Zn deposit thickness in mm | Zn deposit morphology |
|----------|-------------------------|---------------------|----------------------------|-----------------------|
| 1        | 1.47                    | 0                   | 3.2                        | smooth                |
| 2        | 1.48                    | 0                   | 3.5                        | "                     |
| 3        | 1.49                    | 0                   | 4.1                        | "                     |
| 4        | 1.47                    | 0                   | 3.5                        | "                     |
| 5        | 1.48                    | 0                   | 3.1                        | "                     |
| 6        | 1.50                    | 0                   | 3.0                        | "                     |
| 7        | 1.49                    | 0                   | 3.0                        | "                     |
| 8        | 1.50                    | 0                   | 4.1                        | "                     |
| 9        | 1.48                    | 0                   | 4.1                        | "                     |
| 10       | 1.47                    | 0                   | 4.0                        | "                     |

The cathodic current efficiency was found to be 92-95% in all cases and the purity of the zinc deposit was 99.999%.

## EXAMPLE VI

Using the procedure of Example V, 5 titanium plates (20 × 20 cm) were coated with the composition of Example V. The coated plates were used as anodes in a cell for recovery of copper from an aqueous electrolyte containing 100 g/liter (as free metal) of CuSO<sub>4</sub> and 10 g/liter of sulfuric acid and the cathode was a smooth steel plate. The electrolyte gap was 15 mm and the bath temperature was 60°C. The current density was 500 A/m<sup>2</sup>. The anode potential, loss of coating and copper thickness and morphology of the copper deposit are reported in Table IX.

TABLE IX

| Test No. | Anode potential V (NHE) | Coating weight loss | Cu deposit thickness in mm | Cu deposit morphology |
|----------|-------------------------|---------------------|----------------------------|-----------------------|
| 20       | 1                       | 1.47                | 0                          | 4.5                   |
|          | 2                       | 1.50                | 0                          | 4.5                   |
|          | 3                       | 1.48                | 0                          | 5.8                   |
|          | 4                       | 1.47                | 0                          | 4.1                   |
|          | 5                       | 1.49                | 0                          | 5.8                   |

The cathodic current efficiency was found to be 100% in all cases and the purity of the copper was 99.9999%.

## EXAMPLE VII

16 titanium coupons (20 × 20 mm) were etched in boiling azeotropic 20% hydrochloric acid for 40 minutes and were thoroughly washed. The coupons were then coated with the composition of Table X in 20 coats. After the first 19 coats, the coupons were heated in a forced air circulation oven at 500°C and then were air cooled. The last heating was at 500° or 550°C for 1 hour followed by air cooling.

TABLE X

| Specimen No. | Liquid Coating per gm of noble metal/m <sup>2</sup> each titanium sheet coupon |                |    |
|--------------|--------------------------------------------------------------------------------|----------------|----|
| 1,1A,1B,1C   | TaCl <sub>5</sub>                                                              | 2.077 mg as Ta | 16 |
|              | IrCl <sub>3</sub>                                                              | 3.2 mg as Ir   |    |
|              | CaCl <sub>2</sub> ·6H <sub>2</sub> O                                           | 0.053 mg as Ca |    |
|              | HCl                                                                            | 0.0413 mls.    |    |
| 2,2A,2B,2C   | TaCl <sub>5</sub>                                                              | 2.000 mg as Ta | 16 |
|              | IrCl <sub>3</sub>                                                              | 3.2 mg as Ir   |    |
|              | CaCl <sub>2</sub> ·6H <sub>2</sub> O                                           | 0.13 mg as Ca  |    |
|              | HCl                                                                            | 0.0394 mls.    |    |
| 3,3A,3B,3C   | TaCl <sub>5</sub>                                                              | 1.92 mg as Ta  | 16 |
|              | IrCl <sub>3</sub>                                                              | 3.2 mg as Ir   |    |
|              | CaCl <sub>2</sub> ·6H <sub>2</sub> O                                           | 0.21 mg as Ca  |    |
|              | HCl                                                                            | 0.0374 mls.    |    |
| 4,4A,4B,4C   | TaCl <sub>5</sub>                                                              | 1.87 mg as Ta  | 16 |
|              | IrCl <sub>3</sub>                                                              | 3.2 mg as Ir   |    |
|              | CaCl <sub>2</sub> ·6H <sub>2</sub> O                                           | 0.26 mg as Ca  |    |
|              | HCl                                                                            | 0.0362 mls.    |    |

The samples were then tested in 10% sulfuric acid at 60°C with an anodic current density of 1.2 KA/m<sup>2</sup> to determine the anode potential and coating loss after 2500 hours. The results are shown in Table XI.

TABLE XI

| Specimen No. | Temperature final heat treatment | Ca content % b.w.t. | Anode Potential initial value V (NHE) | Anode Potential after 2500 hs. V (NHE) | Weight loss mg/cm <sup>2</sup> |
|--------------|----------------------------------|---------------------|---------------------------------------|----------------------------------------|--------------------------------|
| 1            | 500°C                            | 1                   | 1.51                                  | 1.55                                   | 0                              |
| 1A           | "                                | 1                   | 1.51                                  | 1.56                                   | "                              |
| 1B           | 550°C                            | 1                   | 1.51                                  | 1.56                                   | "                              |
| 1C           | "                                | 1                   | 1.51                                  | 1.56                                   | "                              |
| 2            | 500°C                            | 2.5                 | 1.50                                  | 1.51                                   | "                              |
| 2A           | "                                | 2.5                 | 1.51                                  | 1.51                                   | "                              |
| 2B           | 550°C                            | 2.5                 | 1.50                                  | 1.52                                   | "                              |

TABLE XI-continued

| Specimen No. | Temperature final heat treatment | Ca content % b.w.t. | Anode Potential initial value V(NHE) | Anode Potential after 2500 hs. V(NHE) | Weight loss mg/cm <sup>2</sup> | 5  |
|--------------|----------------------------------|---------------------|--------------------------------------|---------------------------------------|--------------------------------|----|
| 2C           | "                                |                     | 1.50                                 | 1.52                                  | "                              |    |
| 3            | 500°C                            | 4.0                 | 1.51                                 | 1.58                                  | "                              |    |
| 3A           | "                                |                     | 1.52                                 | 1.58                                  | "                              |    |
| 3B           | 550°C                            | 4.0                 | 1.51                                 | 1.55                                  | "                              | 10 |
| 3C           | "                                |                     | 1.51                                 | 1.58                                  | "                              |    |
| 4            | 500°C                            | 5.0                 | 1.51                                 | 1.60                                  | "                              |    |
| 4A           | "                                |                     | 1.52                                 | 1.60                                  | "                              |    |
| 4B           | 550°C                            | 5.0                 | 1.52                                 | 1.65                                  | "                              |    |
| 4C           | "                                |                     | 1.52                                 | 1.65                                  | "                              |    |

## EXAMPLE VIII

Using the procedure of Example VII, 20 × 20mm titanium coupons were coated with the composition of Table XII with the same heatings.

TABLE XII

| Specimen No. | Liquid coating per each titanium sheet coupon |                 |  | N.M. amount gr/m <sup>2</sup> |
|--------------|-----------------------------------------------|-----------------|--|-------------------------------|
| 1.1A,1B,1C   | TaCl <sub>5</sub>                             | 2.077 mg. as Ta |  |                               |
|              | IrCl <sub>3</sub>                             | 3.200 mg. as Ir |  | 16                            |
|              | CoCl <sub>2</sub> .6H <sub>2</sub> O          | 0.053 mg. as Co |  |                               |
|              | HCl                                           | 0.0412 mls.     |  |                               |
| 2.2A,2B,2C*  | TaCl <sub>5</sub>                             | 2.000 mg. as Ta |  |                               |
|              | IrCl <sub>3</sub>                             | 3.200 mg. as Ir |  | 16                            |
|              | CoCl <sub>2</sub> .6H <sub>2</sub> O          | 0.13 mg. as Co  |  |                               |
|              | HCl                                           | 0.0394 mls.     |  |                               |
| 3.3A,3B,3C   | TaCl <sub>5</sub>                             | 1.92 mg. as Ta  |  |                               |
|              | IrCl <sub>3</sub>                             | 3.200 mg. as Ir |  | 16                            |
|              | CoCl <sub>2</sub> .6H <sub>2</sub> O          | 0.21 mg. as Co  |  |                               |
|              | HCl                                           | 0.0374 mls.     |  |                               |
| 4.4A,4B,4C   | TaCl <sub>5</sub>                             | 1.87 mg. as Ta  |  |                               |
|              | IrCl <sub>3</sub>                             | 3.200 mg. as Ir |  | 16                            |
|              | CoCl <sub>2</sub> .6H <sub>2</sub> O          | 0.26 mg. as Co  |  |                               |
|              | HCl                                           | 0.0362 mls.     |  |                               |

The anode potentials and the coating losses after 8000 hours was determined as in Example VII and the results are reported in Table XIII.

TABLE XIII

| Specimen | Temperature final heat treatment | Co content % b.w.t. | Anode Potential initial value V(NHE) | Anode Potential after 8000 hs. V(NHE) | Coating weight loss mg/cm <sup>2</sup> |
|----------|----------------------------------|---------------------|--------------------------------------|---------------------------------------|----------------------------------------|
| 1        | 500°C                            | 1                   | 1.52                                 | 1.56                                  | 0                                      |
| 1A       | "                                | 1                   | 1.52                                 | 1.56                                  | "                                      |
| 1B       | 550°C                            | "                   | 1.52                                 | 1.57                                  | "                                      |
| 1C       | "                                | "                   | 1.52                                 | 1.57                                  | "                                      |
| 2        | 500°C                            | 2.5                 | 1.52                                 | 1.53                                  | "                                      |
| 2A       | "                                | "                   | 1.52                                 | 1.53                                  | "                                      |
| 2B       | 550°C                            | "                   | 1.52                                 | 1.54                                  | "                                      |
| 2C       | "                                | "                   | 1.52                                 | 1.54                                  | "                                      |
| 3        | 500°C                            | 4                   | 1.52                                 | 1.56                                  | "                                      |
| 3A       | "                                | "                   | 1.52                                 | 1.56                                  | "                                      |
| 3B       | 550°C                            | "                   | 1.52                                 | 1.56                                  | "                                      |
| 3C       | "                                | "                   | 1.52                                 | 1.56                                  | "                                      |
| 4        | 500°C                            | 5                   | 1.52                                 | 1.56                                  | "                                      |
| 4A       | "                                | "                   | 1.52                                 | 1.57                                  | "                                      |
| 4B       | 550°C                            | "                   | 1.52                                 | 1.56                                  | "                                      |
| 4C       | "                                | "                   | 1.52                                 | 1.57                                  | "                                      |

Various modifications of the electrodes and processes of the invention may be made without departing from the spirit or scope thereof and it should be understood that the invention is to be limited only as defined in the appended claims.

We claim:

1. A method of electrowinning metals comprising passing an electric current through an anode having an electro-conductive base provided with a coating over at least a portion of its outer surface of a mixed material of tantalum oxide and iridium oxide, then an acid aqueous electrolyte containing the metal to be electrowinned and then the cathode on which the electrowinned metal is deposited, the ratio of tantalum or iridium calculated as metal is 7:1 to 0.34 to 1.
2. The method of claim 1 wherein the electro-conductive base is a valve metal.
3. The method of claim 2 wherein the valve metal is titanium.
4. The method of claim 1 wherein the electro-conductive base is titanium alloyed with up to 0.2% by weight of palladium.
5. The method of claim 1 wherein the coating also contains an oxide of a doping metal selected from the group consisting of alkaline earth metal, cobalt, iron, nickel, chromium, molybdenum and manganese.
6. The method of claim 5 wherein the doping metal is selected from the group consisting of cobalt and calcium.

\* \* \* \* \*

UNITED STATES PATENT OFFICE  
CERTIFICATE OF CORRECTION

Patent No. 3,926,751 Dated December 16, 1975

Inventor(s) Oronzio De Nora et al.

It is certified that error appears in the above-identified patent and that said Letters Patent are hereby corrected as shown below:

Column 3, line 23, "mebers" should read -- members --;  
line 39, "los" should read -- low --. Column 10, line 32,  
"7" should read -- 1 --.

**Signed and Sealed this**  
**Thirteenth Day of July 1976**

**[SEAL]**

*Attest:*

**RUTH C. MASON**  
*Attesting Officer*

**C. MARSHALL DANN**  
*Commissioner of Patents and Trademarks*